# EUROPEAN PATENT SPECIFICATION

(11) **EP 0 912 981 B1**
(45) Date of publication and mention of the grant of the patent: **26.11.2003**
(21) Application number: 97932163.5
(22) Date of filing: 11.06.1997
(51) Int. Cl.: H01B 3/20

(54) **HIGH OLEIC ACID ELECTRICAL INSULATION FLUIDS AND METHOD OF MAKING THE SAME**
ELEKTROISOLIERFLÜSSIGKEITEN MIT EINEM HOHEN GEHALT AN ÖLSÄURE SOWIE VERFAHREN ZU IHRER HERSTELLUNG
FLUIDES ISOLANTS RICHES EN ACIDE OLEIQUE ET PROCEDE DE FABRICATION ASSOCIE

(30) Priority: 18.06.1996 US 665721
(43) Date of publication of application: 06.05.1999
(73) Proprietor: ABB Inc., Raleigh, NC 27606 (US)
(72) Inventor: OOMMEN, Thottathil, V., Raleigh, NC 27606 (US); CLAIBORNE, C., Clair, Sharon, PA 16146 (US)
(74) Representative: W.P. THOMPSON & CO.
(86) International application number: US9710045
(87) International publication number: WO97049100

(56) References cited:
- EP-A- 0 083 736
- EP-A- 0 512 734
- EP-A- 0 714 974
- WO-A-91/02784
- WO-A-97/22977
- JP-A- 52 025 298
- US-A- 323 753
- US-A- 4 536 331
- US-A- 4 627 192
- US-A- 5 260 077
- US-A- 5 336 423
- US-A- 5 429 761
- US-A- 5 538 654
- N SHIGEYOSHI ET ALL: "Electric insulating oil" CHEMICAL ABSTRACTS + INDEXES, vol. 20, no. 105, 17 November 1986, page 190 XP002097870
- N SHIGEYOSHI ET ALL: "Electric insulating oils" CHEMICAL ABSTRACTS + INDEXES, vol. 22, no. 105, 1 December 1986, page 195 XP002097871
- N SHIGEYOSHI: "Oil insulators for electric apparatus" CHEMICAL ABSTRACTS + INDEXES, vol. 14, no. 106, 6 April 1987, page 683 XP002097872
- N SHIGEYOSHI ET ALL: "Oil containing alkyl methacrylate polymers for electrical equipment" CHEMICAL ABSTRACTS + INDEXES, vol. 2, no. 109, 11 July 1988, page 631 XP002097873
- DATABASE WPI Section Ch, Week 8615 Derwent Publications Ltd., London, GB; Class A85, AN 86-097634 XP002097874 & JP 61 042816 A (NICHICON CAPACITOR LTD) , 1 March 1986
- UOP, FOOD PRODUCTS AND PROCESSES, 1994, "Sustane, Food-Grade Antioxidants", pages 3 and 7.

## Description

### FIELD OF THE INVENTION

The invention relates to a high oleic oil composition useful as an electrical insulation fluid, to electrical insulation fluid compositions and electrical apparatuses which comprise the same. The high oleic oil compositions of the invention have electrical properties which make them well suited as insulation fluids in electrical components.

### BACKGROUND OF THE INVENTION

The electrical industry uses a variety of insulating fluids which are easily available and cost effective. Examples are mineral oil, silicone fluid, and synthetic hydrocarbon oils used in transformers, power cables and capacitors. Examples of such fluids include those described in U.S. Patent Number 4,082,866 issued April 4, 1978 to Link, U.S. Patent Number 4,206,066 issued June 3, 1980 to Rinehart, U.S. Patent Number 4,621,302 issued November 4, 1986 to Sato et al., U.S. Patent Number 5,017,733 issued May 21, 1991 to Sato et al. U.S. Patent Number 5,250,750 issued October 5, 1993 to Shubkin et al., and U.S. Patent Number 5,336,847 issued August 9, 1994 to Nakagami.

Many of these fluids are not considered to be biodegradable in a reasonable time frame. Some have electrical properties which render them less than optimal. In recent years regulatory agencies have become increasingly concerned about oil spills which can contaminate the ground soil and other areas. A biodegradable oil would be desirable for electrical apparatus such as transformers used in populated areas and shopping centers.

Vegetable oils are fully biodegradable, but the oils presently available in the market are not electrical grade. A few vegetable oils such as rapeseed oil and castor oil have been used in limited quantities, mostly in capacitors, but these are not oleic esters.

There is a need for a fully biodegradable electrical fluid. There is a need for electrical apparatuses which comprise such an oil. There is a need for a method of processing vegetable oil to electrical grade.

### SUMMARY OF THE INVENTION

The present invention in its broades as well as preferred narrows aspects is defined in the claims, to which reference should now be made.

The present invention can thus provide a high oleic acid triglyceride compositions that comprise fatty acid components of at least 75% oleic acid, less than 10% diunsaturated fatty acid component; less than 3% triunsaturated fatty acid component; and less than 8% saturated fatty acid component;.and wherein said composition is further characterized by the properties of a dielectric strength of at least 35 kV/100 mil gap (35 kV/2.5 mm gap), a dissipation factor of less than 0.05% at 25°C, acidity equal to or less than 0.05 mg KOH/g, electrical conductivity of less than 1 pS/m at 25°C, a flash point of at least 250°C and a pour point of at least -15°C.

The present invention can also provide an electrical insulation fluid comprising at least 75% of a high oleic acid triglyceride composition that comprises fatty acid components of at least 75% oleic acid, less than 10% diunsaturated fatty acid component; less than 3% triunsaturated fatty acid component; and less than 8% saturated fatty acid component; and wherein said composition is further characterized by the properties of a dielectric strength of at least 35 kV/100 mil gap (35 kV/2.5 mm gap), a dissipation factor of less than 0.05% at 25°C, acidity equal to or less than 0.05 mg KOH/g, electrical conductivity of less than 1 pS/m at 25°C, a flash point of at least 250°C and a pour point of at least - 15°C, and one or more additive selected from the group of an antioxidant additive, a pour point depressant additive and a copper deactivator.

The present invention relates to electrical apparatuses comprising the electrical insulation fluid.

The present invention relates to the use of electrical insulation fluid to provide insulation in electrical apparatuses.

### DETAILED DESCRIPTION OF THE INVENTION

This present invention provides a novel application for high oleic vegetable oils as electrical insulation fluids. Vegetable oils usually have a high percent of triglyceride esters of saturated and unsaturated organic acids. When the acid is saturated, the triglyceride is either a semi-solid or a liquid with high freezing point. Unsaturated acids produce oils with low freezing points. However, monounsaturated acids are preferred over diunsaturated and triunsaturated acids because the latter tend to dry fast in air due to cross-linking with oxygen. Increasing the amount of diunsaturates and triunsaturates makes the oil more vulnerable to oxidation; increasing the saturates raises the pour point. Ideally, the higher the monosaturate content, the better the oil as an electrical fluid.

Oleic acid is a monounsaturated acid found as triglyceride ester in many natural oils such as sunflower, olive oil and safflower in relatively high proportions (above 60%). High oleic acid content is usually above 75% of the total acid content. Oleic acid content above 80% is achieved by genetic manipulation and breeding. Two oils that are currently available in the United States with high oleic acid content and low saturates are sunflower oil and canola oil. These oils are of value in producing high quality lubricating oils but have not been used in the production of electrical insulation fluids.

High oleic oils may be derived from plant seeds such as sunflower and canola which have been genetically modified to yield high oleic content. The pure oils are triglycerides of certain fatty acids with a carbon chain ranging from 16 to 22 carbon atoms. If the carbon chain has no double bonds, it is a saturated oil, and is designated Cn:0 where n is the number of carbon atoms. Chains with one double bond are monounsaturated and are designated Cn:1; with two double bonds, it will be Cn:2 and with three double bonds Cn:3. Oleic acid is a C18:1 acid while erucic acid is a C22:1 acid. The acids are in the combined state as triglycerides, and when the oils are hydrolyzed they are separated into the acid and glycerol components. High oleic oils contain more than 75% oleic acid (in combined state with glycerol), the remaining being composed mainly of C18:0, C18:2 and C18:3 acids (also in combined state with glycerol). These acids are known as stearic, linoleic and linolenic. Oils with a high percentage of double and triple unsaturated molecules are unsuitable for electrical application because they react with air and produce oxidation products. Monounsaturated oils such as oleic acid esters may also react with air, but much slower, and can be stabilized with oxidation inhibitors.

A typical 85% high oleic oil has the following approximate composition:

| | |
|---|---|
| Saturates | 3-5% |
| monounsaturates | 84-85% |
| diunsaturates | 3-7% |
| triunsaturates | 1-3% |

While the present invention provides for the use of vegetable oils, the invention may use synthetic oil having the same compositional characteristics of those oils isolated from plants. While plant derived material is suitable for almost all applications, synthetic material may provide a desirable alternative in some applications.

According to the present invention, high oleic acid content oils are used as starting materials for the production of an oil composition which has physical properties useful for electrical insulation fluids. The present invention provides the processed compositions having specific structural and physical characteristics and properties, methods of making such composition, electrical insulation fluids which comprise the composition, electrical apparatuses which comprise the electrical insulation fluids and methods of insulating electrical apparatuses using such fluids.

The present invention provides a high oleic acid triglyceride composition useful as an electrical insulation fluid and more particularly as a component material of an electrical insulation fluid. A triglyceride composition is a glycerol backbone linked to three fatty acid molecules. The triglyceride compositions of the invention comprise fatty acid components of at least 75% oleic acid. The remaining fatty acid components include less than 10% diunsaturated fatty acid component, less than 3% triunsaturated fatty acid component; and less than 8% saturated fatty acid component.

The triglyceride compositions of the invention preferably comprise fatty acid components of at least 80% oleic acid. The triglyceride compositions of the invention more preferably comprise fatty acid components of at least 85% oleic acid. In some embodiments, the triglyceride compositions of the invention comprise fatty acid components of 90% oleic acid. In some embodiments, the triglyceride compositions of the invention comprise fatty acid components of greater than 90% oleic acid.

Di-unsaturated, triunsaturated and saturated fatty acid components present in the triglyceride are preferably C16-C22. It is preferred that 80% or more of the remaining fatty acid components are C18 diunsaturated, triunsaturated and saturated fatty acids, i.e. linoleic, linolenic and stearic acids, respectively. In some embodiments, the diunsaturated, triunsaturated and saturated fatty acid components of the triglyceride comprise at least 75% oleic acid, less than 3% linoleic acid, less than 4% stearic acid and less than 4% palmitic acid (saturated C16).

The triglyceride compositions of the invention are of an electric grade. That is, they have specific physical properties which make them particularly suited for use as an electrical insulation fluid. The dielectric strength of a triglyceride composition of the invention is at least 35 kV/100 mil gap (35 kV/2.5 mm gap), the dissipation factor is less than 0.05% at 25°C, the acidity is equal to or less than 0.05 mg KOH/g, the electrical conductivity is less than 1 pS/m at 25°C, the flash point is at least 250°C and the pour point is at least -15°C.

The dielectric strength, dissipation factor, acidity, electrical conductivity, flash point and pour point are each measured using the published standards set forth in the Annual Book of ASTM Standards (in Volumes 5 and 10) published by the American Society for Testing Materials (ASTM), 100 Barr Harbor Drive West Conshohocken PA 19428. The dielectric strength is determined using ASTM test method D 877. The dissipation factor is determined using ASTM test method D 924. The acidity is determined using ASTM test method D 974. The electrical conductivity is determined using ASTM test method D 2624. The flash point is determined using ASTM test method D 92. The pour point is determined using ASTM test method D 97.

The dielectric strength is measured by taking 100-150 ml oil sample in a test cell and applying a voltage between test electrodes separated by a specified gap. The breakdown voltage is noted. The test is preferably run five times and the average value is calculated. The dielectric strength of a triglyceride composition of the invention is at least 35 kV/100 mil gap (35 kV/2.5 mm gap). In some preferred embodiments, it is 40 kV/100 mil gap (40 kV/2.5 mm gap).

The dissipation factor is a measure of the electrical loss due to conducting species and is tested by measuring the capacitance of fluids in a test cell using a capacitance bridge. The dissipation factor of a triglyceride composition of the invention is less than 0.05% at 25C. In some preferred embodiments, it is less than 0.02%. In some preferred embodiments, it is less than 0.01%.

The acidity is measured by titrating a known volume of oil with a solution of alcoholic KOH to neutralization point. The weight of the oil in grams per mg KOH is referred to interchangeably as the acidity number or the neutralization number. The acidity of a triglyceride composition of the invention is less than 0.03 mg KOH/g. In some preferred embodiments, it is less than 0.02 mg KOH/g.

The electrical conductivity is measured using a conductivity meter such as an Emcee meter. The electrical conductivity of a triglyceride composition of the invention is less than 1 pS/m at 25°C. In some preferred embodiments, it is less than 0.25 pS/m.

The flash point is determined by placing an oil sample in a flashpoint tester and determining the temperature at which it ignites. The flash point of a triglyceride composition of the invention is at least 250°C. In some preferred embodiments, it is at least 300°C.

The pour point is determined by cooling an oil sample with dry ice/acetone and determining the temperature at which the liquid becomes a semi-solid. The pour point of a triglyceride composition of the invention is not greater than -15°C. In some preferred embodiments, it is not greater than -20°C. In some preferred embodiments, it is not greater than -40°C.

In some preferred embodiments, the triglyceride composition of the invention is characterized by the properties of a dielectric strength of at least 40 kV/100 mil gap (40 kV/2.5 mm gap), a dissipation factor of less than 0.02% at 25°C, acidity of less than 0.02 mg KOH/g, electrical conductivity of less than 0.25 pS/m at 25°C, a flash point of at least 300°C and a pour point of not greater than -20°C. In some preferred embodiments, the pour point is not greater than -40°C.

In some preferred embodiments, the triglyceride composition of the invention comprises fatty acid components of at least 75% oleic acid, linoleic acid at a proportion of less than 10%, linoleic acid at a proportion of less than 3%, stearic acid in a proportion of less than 4%, and palmitic acid in a proportion of less than 4%, and is characterized by the properties of a dielectric strength of at least 40 kV/100 mil gap (40 kV/2.5 mm gap), a dissipation factor of less than 0.02% at 25°C, acidity of less than 0.02 mg KOH/g, electrical conductivity of less than 0.25 pS/m at 25°C, a flash point of at least 300°C and a pour point of not greater than -20°C. In some preferred embodiments, the pour point is not greater than -40°C.

Triglycerides with high oleic acid oil content are described in U.S. Patent Number 4,627,192 issued December 4, 1986 to Fick and U.S. Patent Number 4,743,402 issued May 10, 1988 to Fick. These oils or those with similar fatty acid component content according to the present invention may be processed to yield an oil with the desired physical properties. High oleic vegetable oils may be obtained from commercial suppliers as RBD oils (refined, bleached and deodorized) which are further processed according to the present invention to yield high oleic oils useful in electrical insulation fluid compositions. There are several suppliers of high oleic RBD oils in the USA and overseas. RBD oil useful as a starting material for further processing may be obtained from SVO Specialty Products, Eastlake OH, and Cargill Corp., Minneapolis MN. The oil manufacturer goes through an elaborate process to obtain RBD oil during which all nonoily components (gums, phospholipids, pigments etc.) are removed. Further steps may involve winterization (chilling) to remove saturates, and stabilization using nontoxic additives. The processes for converting oil to RBD oil are described in Bailey's Industrial Oil and Fat Products, Vols. 1, 2 & 3, Fourth Edition 1979 John Wiley & Sons. and in Bleaching and Purifying Fats and Oils by H.B.W. Patterson, AOCC Press, 1992.

RBD oils are further processed according to the present invention in order to yield an oil with the physical properties as defined herein. The purification of the as received oil designated RBD oil is necessary because trace polar compounds and acidic materials still remain in the oil, making it unfit as an electrical fluid. The purification process of the present invention uses clay treatment which involves essentially a bleaching process using neutral clay. RBD oil is combined with 10% by weight clay and mixed for at least about 20 minutes. It is preferred if the oil is heated to about 60-80°C. It is preferred if the mixture is agitated. The clay particles are removed subsequently by a filter press. Vacuum conditions or a neutral atmosphere (by nitrogen) during this process prevent oxidation. Slightly stabilized oil is preferable. More stabilizer is added at the end of the process. The purity is monitored by electrical conductivity, acidity and dissipation factor measurement. Further treatment by deodorization techniques is possible but not essential. The polar compounds that interfere most with electrical properties are organometallic compounds such as metallic soaps, chlorophyll pigments and so on. The level of purification needed is determined by the measured properties and the limits used. An alternative embodiment provides passing RBD oil through a clay column. However, stirring with clay removes trace polar impurities better than passing through a clay column. In preferred embodiments, neutral Attapulgite clay, typically 30/60 mesh size, is used in a ratio of 1-10% clay by weight. In some embodiments, clay particles are removed using filters, preferably paper filters with a pore size of 1-5 µm. The clay is preferably mixed with hot oil and agitated for several minutes, after which the clay is filtered off using filters. Paper or synthetic filter sheets may be used if a filter separator is used. The filter sheets are periodically replaced.

Electrical insulation fluids of the invention comprise the triglyceride composition of the invention and may further comprise one or more additives. Additives include oxidation inhibitors, copper deactivators and pour point depressors.

Oxidation inhibitors may be added to the oils. Oxidation stability is desirable but in sealed units where there is no oxygen, it should not be critical. Commonly used oxidation inhibitors include butylated hydroxy toluene (BHT), butylated hydroxy anisole (BHA) and mono-tertiary-butyl-hydroquinone (TBHQ). In some embodiments, oxidation inhibitors are used in combinations such as BHA and BHT. Oxidation inhibitors may be present at levels of 0.1-3.0%. In some preferred embodiments, 0.2% TBHQ is used. Oxidation stability of the oil is determined by AOM or OSI methods well known to those skilled in the art. In the AOM method, the oil is oxidized by air at 100°C and the formation of peroxide is monitored. The time to reach 100 milliequivalents (meq) or any other limit is determined. The higher the value, the more stable the oil is. In the OSI method, the time to reach an induction period is determined by the measurement of conductivity.

Pour points depressants may also be added if low pour points are needed. Commercially available products can be used which are compatible with vegetable-based oils. Only low percentages, such as 2% or below, are needed normally to bring down the pour point by 10 to 15°C. In some embodiments, the pour point depressant is polymethacrylate (PMA).

Since copper is always present in the electrical environment, another type of additive is copper deactivators. Copper deactivators such as benzotriazole derivatives are commercially available. The use of these in small, such as below 1%, may be beneficial in reducing the catalytic activity of copper in electrical apparatus. In some embodiments, the electrical insulation fluid contains less than 1% of a copper deactivator. In some embodiments, the copper deactivator is a benzotriazole derivative.

In some embodiments, the pour point may be further reduced by winterizing processed oil. Essentially, the oils are winterized by lowering the temperature to near or below 0°C and removing solidified components. The winterization process may be performed as a series of temperature reductions followed by removal of solids at the various temperature. In some embodiments, winterization is performed by reducing the temperature serially to 5°, 0° and -12°C for several hours, and filtering the solids with diatomaceous earth.

In some embodiments, the electrical insulation fluid of the invention that comprises at least 75 percent triglyceride composition of the invention as described above further comprises about 0.1-5% additives and then up to about 25% other insulating fluids such as mineral oil, synthetic esters, and synthetic hydrocarbons. In some embodiments, the electrical insulation fluid comprises 1-24% of insulating fluids selected from the group consisiting of mineral oil, synthetic esters, synthetic hydrocarbons and combinantion of two or more of such materials. In some embodiments, the electrical insulation fluid comprises 5-15% of insulating fluids selected from the group consisiting of mineral oil, synthetic esters, synthetic hydrocarbons and combinantion of two or more of such materials. Examples of mineral oils include poly alpha olefins. An example of a mineral oil which may be used as part of the present invention is RTEemp, Cooper Power Fluid Systems. Examples of synthetic esters include polyol esters. Commercially available synthetic esters which can be used as part of the invention include those sold under the trade names MYDEL, REODEC and ENVIROTEMP 200, Cooper Power Fluid Systems. In some preferred embodiments, the electrical insulation fluid comprises at least 85% of the triglyceride composition of the invention. In some preferred embodiments, the electrical insulation fluid comprises at least 95% of the triglyceride composition of the invention.

The present invention relates to an electrical apparatus which comprises the electrical insulation fluid of the invention. The electrical apparatus may be an electrical transformer, an electrical capacitor or an electrical power cable. U.S. Patent Number 4,082,866, U.S. Patent Number 4,206,066, U.S. Patent Number 4,621,302, U.S. Patent Number 5,017,733, U.S. Patent Number 5,250,750, and U.S. Patent Number 5,336,847 describe various applications of electrical insulation fluids for which the electrical insulation fluid of the invention may be used. In addition, U.S. Patent Number 4,993,141 issued February 19, 1991 to Grimes et al., U.S. Patent Number 4,890,086 issued December 26, 1989 to Hill, U.S. Patent Number 5,025,949 issued June 25, 1991 to Adkins et al., U.S. Patent Number 4,972,168 issued November 20, 1990 to Grimes et al., U.S. Patent Number 4,126,844, and U.S. Patent Number 4,307,364 issued December 22, 1981 to Lanoue et al. contain descriptions of various electrical apparatuses in which the electrical insulation fluid of the invention may be used. In some preferred embodiments, the eletrical apparatus fo the invention is a transformer, in particular,a power transformer or a distribution transformer.

### EXAMPLES

### Example 1

Several high oleic oils were further purified and stabilized according to the present invention to make them electrically suitable. Electrical tests showed that such purified oils had properties similar to currently used high temperature fluids in distribution transformers. Table 1 compares the properties of the purified oils of the present invention with currently used fluids.

**Table 1**

| Comparison of Purified Vegetable Oils with High Temperature Fluids Used in Transformers | | | |
|---|---|---|---|
| | High Oleic Veg. Oil | High Temp. Mineral Oil^{a} | Synthetic Ester Fluid^{b} |
| Dielectric Strength, KV/100 mil gap | 42.4 | 40-45 | 50 |
| Dissipation Factor, % at 25°C | 0.02 | 0.01 | 0.1 |
| Neutr. No. mg KOH/g | 0.05 | - | 0.03 |
| Electrical Conductivity pS/m, 25°C | 0.25-1.0 | (0.1 o 10)* | (5.0)* |
| Flash Point | 328°C | 275-300°C | 257°C |
| Pour Point | -28°C | -24°C | -48° |

| | | | |
|---|---|---|---|
| ^{a} RTEemp, Cooper Power Fluid Systems | | | |
| ^{b} Polyol Esters | | | |
| * deduced from resistivity | | | |

The properties listed for the high oleic oil are for purified oils with no additives.

### Example 2

The purification of the as received oil designated RBD oil (refined, bleached and deodorized) is necessary because trace polar compounds and acidic materials still remain in the oil, making it unfit as an electrical fluid. The purification we attempted involved clay treatment as follows: approximately 1 gal. (3.8 l) of the RBD oil was treated with 10% Attapulgite clay. Oil was produced with electrical conductivity of less than 1 pS/m. The attapulgite treated oil showed conductivities as low as 0.25 pS/m. Commercial grade oils had conductivities in the range of 1.5 to 125 pS/m. Conductivity below 1 pS/m (or resistivity above 10¹⁴ ohm.cm) is desired for electrical grade oil. Other indicators of purity are dissipation factor and neutralization number (acid number). Dissipation factor is a measure of electrical losses due to conduction caused by conducting species, usually organometallic trace components, and should be below 0.05% at room temperature. The clay treated oils had dissipation factor of 0.02%. Untreated RBD oils had DF ranging from 0.06% to 2.0%.

### Example 3

Oxidation stability tests were conducted on treated and untreated oil samples using ASTM and AOCS methods. The untreated and treated RBD oils failed the tests. Oxidation inhibitors were added to the oils and the tests were repeated. Several oxidation inhibitors were tested: BHT (Butylated Hydroxy Toluene, BHA (Butylated Hydroxy Anisole) and TBHQ (mono-Tertiary-Butyl-Hydroquinone) in 0.2% by weight in oil. In the AOCS method used (Cd 12.57) 100 ml samples are bubbled with air at 100C, and the peroxide formation was measured at several time intervals. Hours to reach 100 meq of peroxide were noted. Since copper is always present in the electrical environment, all oil samples had copper wire placed in them. With no additive, the time to reach the limit was 18 hours; with additive (0.2%), the times were 100 hours for BHT + BHA. With TBHQ, even after 400 hours, the peroxide value reached only 8.4 meq. TBHQ proved to be the best antioxidant of the three. Without an oxidation inhibitor the oils upon oxidation would produce hydroperoxide which is then converted to acids, alcohols, esters, aldehydes, ketones and polymer structures. Most electrical apparatus that use a fluid insulation operate in low oxygen or oxygen-free environment, so the concern over oxidation is not great.

### Example 4

The pour point of the treated oil was typically -25°C. To lower the pour point further, the treated oils were winterized at 5°, 0° and -12°C for several hours, and the solids that separated were filtered with diatomaceous earth. The lowest pour point reached so far was -38°C, close to the specified value of -40°C for transformer oil. Further lowering is possible by extended winterization. Another approach is by the use of pour point depressants such as PMA (polymethacrylate) which has been used for mineral oil.

## Claims

1. A high oleic acid triglyceride composition comprising fatty acid components of
at least 75% oleic acid
less than 10% diunsaturated fatty acid component C16-C22;
less than 3% triunsaturated fatty acid C16-C22 component; and
less than 8% saturated fatty acid component C16-C22; and
wherein said composition is further **characterized by** the properties of :
a dielectric strength of at least 35 kV/100 mil gap (35 kV/2.5 mm gap)
a dissipation factor of less than 0.05% at 25°C
acidity equal to or less than 0.05 mg KOH/g
electrical conductivity of less than 1 pS/m at 25°C
a flash point of at least 250°C and
a pour point of at least -15°C.

2. A high oleic acid triglyceride composition according to claim 1, comprising fatty acid components of
at least 75% oleic acid
less than 10% linoleic acid
less than 3% linolenic acid
less than 4% stearic acid, and
less than 4% palmitic acid.

3. A high oleic acid triglyceride composition according to claim 1 or 2, wherein said corporation is further **characterized by** an acidity of less than 0.03 mg KOH/g.

4. A high oleic acid triglyceride composition according to claim 2, wherein said composition is further **characterized by** the properties of:
a dielectric strength of at least 40 kV/100 mil gap (40 kV/2.5 mm gap),
a dissipation factor of less than 0.02% at 25°C,
acidity of less than 0.02 mg KOH/g,
electrical conductivity of less than 0.25 pS/m at 25°C,
a flash point of at least 300°C, and
a pour point of at least -20°C.

5. A high oleic acid triglyceride composition according to claim 4, wherein said composition is further **characterized by** a pour point of at least -40°C.

6. A high oleic acid triglyceride composition according to claim 1, comprising fatty acid components of
at least 75% oleic acid
less than 10% linoleic acid
less than 3% linolenic acid
less than 4% stearic acid, and
less than 4% palmitic acid
wherein said composition is further **characterized by** the properties of:
a dielectric strength of at least 40 kV/100 mil gap (40 kV/2.5 mm gap)
a dissipation factor of less than 0.02% at 25°C,
acidity of less than 0.02 mg KOH/g,
electrical conductivity of less than 0.25 pS/m at 25°C,
a flash point of at least 300°C, and
a pour point of at least -20°C.

7. A high oleic acid triglyceride composition according to claim 6, wherein said composition is further **characterized by** a pour point of at least -40°C.

8. An electrical insulation fluid comprising:
at least 75% of the high oleic acid triglyceride composition of claim 1
0.1-3% antioxidant additive.

9. An electrical insulation fluid according to claim 8, wherein said antioxidant additive is selected from the group consisting of butylated hydroxy toluene, butylated hydroxy anisole and mono-t-butyl hydroquinone.

10. An electrical insulation fluid according to claim 8, wherein said antioxidant additive is mono-t-butyl-hydroquinone.

11. An electrical insulation fluid according to claim 10, comprising up to 2% mono-t-butyl-hydroquinone.

12. An electrical insulation fluid according to claim 8, comprising at least 94% of the high oleic acid triglyceride composition.

13. An electrical insulation fluid according to claim 8, further comprising a pour point depressant additive.

14. An electrical insulation fluid according to claim 13, wherein said pour point depressant is polymethacrylate.

15. An electrical insulation fluid according to claim 8, further comprising a copper deactivator additive, said electrical insulation fluid comprising less than 1% of said copper deactivator.

16. An electrical insulation fluid according to claim 8, wherein said copper deactivator is a benzotriazole derivative.

17. An electrical insulation fluid according to claim 8, further comprising up to 25% of mineral oil, synthetic esters, synthetic hydrocarbons and combinantions thereof.

18. A high oleic acid triglyceride composition according to claim 2, wherein said composition is further **characterised by** the property of:
acidity of less than 0.02 mg KOH/g

19. An electrical insulation fluid according to any of claims 8 to 17 containing at least 94% of the said triglyceride composition.

20. An electrical apparatus comprising the electrical insulation fluid of any of claims 8 to 17.

21. An electrical apparatus according to claim 20 wherein said apparatus is an electrical transformer, an electrical capacitor or an electrical power cable.

## Patentansprüche

1. Triglyceridzusammensetzung mit einem hohen Gehalt an Ölsäure, die Fettsäurekomponenten von mindestens 75 % Ölsäure, weniger als 10 % zweifach ungesättigte Fettsäurekomponente C16-C22;
weniger als 3 % dreifach ungesättigte Fettsäurekomponente C16-C22; und
weniger als 8 % gesättigte Fettsäurekomponente C16-C22 enthält und wobei die Zusammensetzung weiterhin durch die folgenden Eigenschaften gekennzeichnet ist:
eine dielektrische Durchschlagsfestigkeit von mindestens 35 kV / 2,5 mm Lücke
einen dielektrischen Verlustfaktor von weniger als 0,05 % bei 25°C
eine Acidität gleich oder weniger als 0,05 mg KOH/g
eine elektrische Leitfähigkeit von weniger als 1 pS/m bei 25°C
einen Flammpunkt von mindestens 250°C und
einen Stockpunkt von mindestens -15°C.

2. Triglyceridzusammensetzung mit einem hohen Gehalt an Ölsäure nach Anspruch 1, die Fettsäurekomponenten von
mindestens 75 % Ölsäure,
weniger als 10 % Linolsäure,
weniger als 3 % Linolensäure,
weniger als 4 % Stearinsäure, und
weniger als 4 % Palmitinsäure enthält.

3. Triglyceridzusammensetzung mit einem hohen Gehalt an Ölsäure nach Anspruch 1 oder 2 , wobei die Zusammensetzung weiterhin **gekennzeichnet ist durch** die Acidität von weniger als 0,03 mg KOH/g.

4. Triglyceridzusammensetzung mit einem hohen Gehalt an ölsäure nach Anspruch 2, wobei die Zusammensetzung weiterhin durch die folgenden Eigenschaften gekennzeichnet ist:
die dielektrische Durchschlagsfestigkeit von mindestens 40 kV / 2,5 mm Lücke,
dem Verlustfaktor von weniger als 0,02 % bei 25°C,
die Acidität von weniger als 0,02 mg KOH/g,
die elektrische Leitfähigkeit kleiner als 0,25 pS/m bei 25°C,
der Flammpunkt mindestens 300°C und
der Stockpunkt mindestens -20°C.

5. Triglyceridzusammensetzung mit einem hohen Gehalt an Ölsäure nach Anspruch 4, wobei die Zusammensetzung weiterhin **dadurch gekennzeichnet ist, daß** der Stockpunkt mindestens -40°C ist.

6. Triglyceridzusammensetzung mit einem hohen Gehalt an Ölsäure nach Anspruch 1, die Fettsäurekomponenten von
mindestens 75 % Ölsäure,
weniger als 10 % Linolsäure,
weniger als 3 % Linolensäure,
weniger als 4 % Stearinsäure, und
weniger als 4 % Palmitinsäure enthält,
wobei die Zusammensetzung durch folgende Eigenschaften weiterhin gekennzeichnet ist:
eine dielektrische Durchschlagsfestigkeit von mindestens 4 0 kV / 2,5 mm Lücke,
einen Verlustfaktor von weniger als 0,02 % bei 25°C,
eine Acidität von weniger als 0, 02 mg KOH/g,
eine elektrische Leitfähigkeit von weniger als 0,25 pS/m bei 25°C,
einen Flammpunkt von mindestens 300°C, und
einen Stockpunkt von mindestens -20°C.

7. Triglyceridzusammensetzung mit einem hohen Gehalt an Ölsäure nach Anspruch 6, wobei die Zusammensetzung weiterhin **gekennzeichnet ist durch** einen Stockpunkt von mindestens -40°C.

8. Elektrische Isolierflüssigkeit, die mindestens 75 % von einer Triglyceridzusammensetzung mit einem hohen Gehalt an Ölsäure nach Anspruch 1, 0,1 - 3 % eines Antioxidantzusatzes enthält.

9. Elektrische Isolierflüssigkeit nach Anspruch 8, wobei der Antioxidantzusatz von einer Gruppe, die butyliertes Hydroxytoluol, butyliertes Hydroxyanisol und Mono-tbutyl-hydrochinon beinhaltet, ausgewählt ist.

10. Elektrische Isolierflüssigkeit nach Anspruch 8, wobei der Antioxidantzusatz Mono-t-butyl-hydrochinon ist.

11. Elektrische Isolierflüssigkeit nach Anspruch 10, die bis zu 2 % Mono-t-butyl-hydrochinon umfaßt.

12. Elektrische Isolierflüssigkeit nach Anspruch 8, **dadurch gekennzeichnet, daß** mindestens 94 % von der Triglyceridzusammensetzung mit einem hohen Gehalt an Ölsäure enthalten ist.

13. Elektrische Isolierflüssigkeit nach Anspruch 8, **dadurch gekennzeichnet, daß** weiterhin ein den Stockpunkt senkender Zusatz enthalten ist.

14. Elektrische Isolierflüssigkeit nach Anspruch 13, wobei der Stockpunktsenker ein Polymethacrylat ist.

15. Elektrische Isolierflüssigkeit nach Anspruch 8, die weiterhin einen Kupferdeaktivatorzusatz enthält, wobei die elektrische Isolierflüssigkeit weniger als 1 % des Kupferdeaktivators enthält.

16. Elektrische Isolierflüssigkeit nach Anspruch 8, wobei der Kupferdeaktivator ein Benzotriazolderivat ist.

17. Elektrische Isolierflüssigkeit nach Anspruch 8, die weiterhin bis zu 25 % Mineralöl, synthetische Ester, synthetische Kohlenwasserstoffe und Kombinationen daraus enthält.

18. Triglyceridzusammensetzung mit einem hohen Gehalt an Ölsäure nach Anspruch 2, wobei die Zusammensetzung durch die folgende Eigenschaft weiterhin gekennzeichnet ist:
Acidität kleiner als 0,02 mg KOH/g.

19. Elektrische Isolierflüssigkeit nach einem der Ansprüche 8 bis 17, die mindestens 94 % der Triglyceridzusammensetzung beinhaltet.

20. Elektrische Vorrichtung, die eine elektrische Isolierflüssigkeit nach einem der Ansprüche 8 bis 17 aufweist.

21. Elektrische Vorrichtung nach Anspruch 20, wobei die Vorrichtung ein elektrischer Transformator, ein elektrischer Kondensator oder ein elektrisches Stromkabel ist.

## Revendications

1. Composition triglycéride riche en acide oléique comprenant des composants d'acide gras de :
au moins 75% d'acide oléique ;
moins de 10% de composant d'acide gras di-insaturé en C16-C22 ;
moins de 3% de composant d'acide gras tri-insaturé en C16-C22 ; et
moins de 8% de composant d'acide gras saturé en C16-C22 ; et
dans laquelle ladite composition est en outre **caractérisée par** les propriétés suivantes :
une rigidité diélectrique d'au moins 35 kV / 100 mil espaces (35 kV / espace de 2,5 mm) ;
un facteur de dissipation inférieur à 0,05% à 25°C ;
une acidité égale à ou inférieure à 0,05 mg KOH / g ;
une conductivité électrique inférieure à 1 pS / m à 25°C ;
un point éclair d'au moins 250°C ; et
un point de figeage d'au moins -15°C.

2. Composition triglycéride riche en acide oléique selon la revendication 1, comprenant les composants d'acide gras de :
au moins 75% d'acide oléique ;
moins de 10% d'acide linoléique ;
moins de 3% d'acide linoléique ;
moins de 4% d'acide stéarique ; et
moins de 4% d'acide palmitique.

3. Composition triglycéride riche en acide oléique selon la revendication 1 ou 2, dans laquelle ladite composition est **caractérisée en outre par** une acidité inférieure à 0,03 mg KOH / g.

4. Composition triglycéride riche en acide oléique selon la revendication 2, dans laquelle ladite composition est **caractérisée en outre par** les propriétés suivantes :
une rigidité diélectrique d'au moins 40 kV / 100 mil espaces (40 kV / espace de 2,5 mm) ;
un facteur de dissipation inférieur à 0,02% à 25°C ;
une acidité inférieure à 0,02 mg KOH / g ;
une conductivité électrique inférieure à 0,25 pS / m à 25°C ;
un point éclair d'au moins 300°C ; et
un point de figeage d'au moins -20°C.

5. Composition triglycéride riche en acide oléique selon la revendication 4, dans laquelle ladite composition est en outre **caractérisée par** un point de figeage d'au moins -40°C.

6. Composition triglycéride riche en acide oléique selon la revendication 1, comprenant les composants d'acide gras suivants :
au moins 75% d'acide oléique ;
moins de 10% d'acide linoléique ;
moins de 3% d'acide linoléique ;
moins de 4% d'acide stéarique ; et
moins de 4% d'acide palmitique
dans laquelle ladite composition est **caractérisée en outre par** les propriétés suivantes :
une rigidité diélectrique d'au moins 40 kV / 100 mil espaces (40 kV / espace de 2,5 mm) ;
un facteur de dissipation inférieur à 0,02% à 25°C ;
une acidité inférieure à 0,02 mg KOH / g ;
une conductivité électrique inférieure à 0,25 pS / m à 25°C ;
un point éclair d'au moins 300°C ; et
un point de figeage d'au moins -20°C.

7. Composition triglycéride riche en acide oléique selon la revendication 6, dans laquelle ladite composition est en outre **caractérisée par** un point de figeage d'au moins -40°C.

8. Fluide d'isolation électrique comprenant :
au moins 75% de la composition triglycéride riche en acide oléique de la revendication 1 ;
0,1 à 3% d'un additif antioxydant.

9. Fluide d'isolation électrique selon la revendication 8, dans lequel ledit additif antioxydant est choisi dans le groupe comprenant l'hydroxytoluène butylé, l'hydroxyanisole butylé et la mono-t-butyl-hydroquinone.

10. Fluide d'isolation électrique selon la revendication 8, dans lequel ledit additif antioxydant est de la mono-t-butyl hydroquinone.

11. Fluide d'isolation électrique selon la revendication 10, comprenant jusqu'à 2% de mono-t-butyl-hydroquinone.

12. Fluide d'isolation électrique selon la revendication 8 comprenant au moins 94% de la composition triglycéride riche en acide oléique.

13. Fluide d'isolation électrique selon la revendication 8, comprenant en outre un additif de dépression du point de figeage.

14. Fluide d'isolation électrique selon la revendication 13, dans lequel ledit agent de dépression du point de figeage est le polyméthacrylate.

15. Fluide d'isolation électrique selon la revendication 8, comprenant en outre un additif de désactivation du cuivre, ledit fluide d'isolation électrique comprenant moins de 1% dudit agent de désactivation du cuivre.

16. Fluide d'isolation électrique selon la revendication 8, dans lequel ledit agent de désactivation du cuivre est un dérivé du benzotriazole.

17. Fluide d'isolation électrique selon la revendication 8, comprenant'en outre jusqu'à 25% d'une huile minérale, d'esters synthétiques, d'hydrocarbures synthétiques et de mélanges de ces éléments.

18. Composition triglycéride riche en acide oléique selon la revendication 2, dans laquelle la composition est **caractérisée en outre par** les propriétés suivantes :
une acidité inférieure à 0,02 mg KOH / g.

19. Fluide d'isolation électrique selon l'une quelconque des revendications 8 à 17 contenant au moins 94% de ladite composition triglycéride.

20. Appareil électrique comprenant le fluide d'isolation électrique de l'une quelconque des revendications 8 à 17.

21. Appareil électrique selon la revendication 20 dans lequel ledit appareil est un transformateur électrique, un condensateur électrique ou un câble de courant électrique.
